

## UNITED STATES PATENT OFFICE

1,925,641

LIGHT PRODUCING IGNITIBLE  
COMPOSITIONStanley Hector Lucas, Witton, Birmingham,  
England, assignor to Imperial Chemical In-  
dustries Limited, a corporation of Great BritainNo Drawing. Application July 7, 1932, Serial No.  
621,314, and in Great Britain October 21,  
1931

7 Claims. (Cl. 52—24)

This invention relates to improvements in compositions which when ignited emit a brilliant light and which consist of a metallic powder mixed with an oxidizing agent. Such compositions consist essentially of one or more finely divided metals such as magnesium, aluminium and zirconium, and oxidizing agents such as potassium chlorate, barium nitrate, potassium nitrate, barium peroxide and the like. These light producing ignitable powders find application in the art of pyrotechny, as flash powders for photographic purposes, and they are also applied for obtaining tracing effects in military and other forms of ammunition. The compositions hitherto used have had certain disadvantages, such as the sensitivity to shock or friction associated with those containing potassium chlorate as the oxidizing agent. Others containing barium peroxide as the oxidizing agent are unstable and suffer deterioration when exposed to the atmosphere. Those containing nitrates are difficult to ignite, and further, barium salts are toxic and therefore undesirable under certain conditions of use, e. g. in connection with tracer pellets for shot gun cartridges.

The objects of this invention are to produce an improved light emitting ignitable composition which is not sensitive to ignition by shock or friction, which is stable when exposed to the atmosphere, which is easily ignitable and non toxic.

I have found that these objects are obtained if the oxidizing agent used in combination with the metallic powder is bismuth oxide or sodium bismuthate or mixtures of these two compounds. Sodium bismuthate is an oxidizing agent and details of its preparation and properties are given in volume 9 of Mellor's "Comprehensive Treatise on Inorganic and Theoretical Chemistry."

Bismuth oxide is preferable to sodium bismuthate since experience has shown that the compositions containing sodium bismuthate, although stable in ordinary atmospheres, are apt to be affected by excess of moisture or exposure to a humid atmosphere for long periods. It appears that under these conditions the sodium bismuthate reacts with the metallic powder, e. g. magnesium, and the ignitability of the composition is thereby impaired. Bismuth oxide, however, does not behave in this way.

It has also been found that the metallic pow-

ders themselves tend to deteriorate when exposed to moisture for long periods and that it is therefore desirable, in order to obtain an absolutely reliable product, to pack the same in air-tight containers. Accordingly, in the manufacture of tracer pellets for ammunition, the composition may be pressed into moisture-proof capsules, the open ends of which are sealed by means of metal foil so that the pellets are completely air and moisture tight.

As an example of one improved light emitting composition prepared in accordance with the invention, I may mention a mixture of two parts of magnesium powder and three parts of bismuth oxide, which when pressed under a load of ten cwts. into tracer pellets for shot gun cartridges, gives excellent results, having the desired properties of certainty of ignition, brightness of trace, and freedom from danger of possible toxic effects. Similar results are obtained with a mixture of one part magnesium powder and one to two parts of sodium bismuthate.

As a further example I may mention a composition containing three parts of bismuth oxide, two parts of magnesium powder or other suitable metallic powder, and half a part of strontium peroxide. The addition of the strontium peroxide changes the white colour of the flame emitted by the tracing composition to a reddish colour and in brilliant sunlight the trace is much more discernible than a completely white light.

While I have referred principally to the use of the improved compositions in connection with tracer pellets for shot gun cartridges, it is to be understood that they are also applicable for a variety of other purposes such as those mentioned in the opening paragraph.

As many apparently widely different embodiments of this invention may be made without departing from the spirit and scope thereof, it is to be understood that I do not limit myself to the specific embodiments thereof except as defined in the appended claims.

I claim:

1. A light-emitting ignitable composition comprising an ignitable metallic powder and bismuth oxide.
2. A light-emitting ignitable composition comprising an ignitable metallic powder and sodium bismuthate.

3. A light-emitting ignitable composition comprising an ignitable metallic powder, bismuth oxide and sodium bismuthate.
4. A light-emitting ignitable composition comprising magnesium powder and bismuth oxide.
5. A light-emitting ignitable composition comprising magnesium powder and sodium bismuthate.

10

6. A light emitting ignitable composition consisting of two parts by weight of magnesium powder and three parts of bismuth oxide.

7. A light-emitting ignitable composition consisting of one part by weight of magnesium powder and 1-2 parts of sodium bismuthate. 80

STANLEY HECTOR LUCAS.

15

85

20

90

25

95

30

100

35

105

40

110

45

115

50

120

55

125

60

130

65

135

70

140

75

145